

Oct. 13, 1925.

1,556,990

R. L. HENRY

COMMUTATOR BRUSH

Filed Oct. 12, 1922



INVENTOR.  
*Ralph L. Henry,*  
BY  
*Fraenkel and Richards,*  
ATTORNEYS.

Patented Oct. 13, 1925.

1,556,990

# UNITED STATES PATENT OFFICE.

RALPH L. HENRY, OF BROOKLYN, NEW YORK, ASSIGNOR TO ALBERT C. HENRY, OF INWOOD, LONG ISLAND, NEW YORK.

## COMMUTATOR BRUSH.

Application filed October 12, 1922. Serial No. 594,088.

To all whom it may concern:

Be it known that I, RALPH L. HENRY, a citizen of the United States, residing at Brooklyn, in the county of Kings and State of New York, have invented certain new and useful Improvements in Commutator Brushes; and I do hereby declare the following to be a full, clear, and exact description of the invention, such as will enable others skilled in the art to which it appertains to make and use the same, reference being had to the accompanying drawings, and to characters of reference marked thereon, which form a part of this specification.

This invention relates, generally, to brushes and contacts for electrical machines, generators, motors and the like, and to a method of manufacturing the same. The invention has for its principal object to provide a novel brush or contact made of a mixture of electrically conductive material, such as graphite, pulverized metals, carbon, coke, lamp-black or other suitable conductive material, combined with a binder of electrically non-conductive or high resistance material, such as a condensation product resulting from the reaction of formaldehyde upon phenol or a phenolic body, or other resinous gum, to provide a material similar to that commonly known as bakelite, redmanol, condensite, etc., or any other form of condensation or other product which has the property of becoming insoluble and infusible when subject to the action of heat.

Said conductive material and non-conductive or high resistance binder material are united by pressure and heat. The pressure is applied in a direction substantially at right angles to the path of least electrical resistance it is desired to be established in the finished brush or contact body; whereby a finished product of desired shape is produced, which possesses a novel physical formation or internal structure adapted to establish a path of least electrical resistance throughout the same along predetermined lines, said lines being usually substantially parallel to the longitudinal axis of the body thus formed; while at the same time the electrical resistance of the body along lines perpendicular to such established path of least resistance is considerably increased, so that the novel physical and electrical char-

acteristics of the finished brush or contact body involves a selective property, highly 55 and especially desirable in commutation in connection with electrical machines, for the body thus offers comparatively low resistance to the flow of main currents through the same to and from the machine, while 60 maintaining a comparatively high resistance to the flow of the commutating, cross, short circuited or internal eddy currents, with the result that the efficiency of commutating machines is greatly increased. 65

In the present invention I do not lay claim broadly to a combination of the aforesaid materials generally for all purposes, but am concerned with a certain procedure and the employment of certain proportions, 70 whereby I am enabled to produce an electrical brush or contact having novel electrical properties, so that the same is characterized by the possession of a path of least electrical resistance along predetermined 75 lines and directions, and comparatively high electrical resistance in directions perpendicular to said predetermined path of least resistance.

The accompanying drawing shows a dia- 80 grammatic perspective of a commutator brush possessing the novel physical and electrical characteristics in accordance with the principles of this invention.

Thus I may proceed as follows. I take 85 graphite, for example, as the conductive material, and a suitable condensation product of the kind above mentioned as the non-conductive or high resistance binder. To nine (9) parts by weight of graphite is added 90 one (1) part by weight of binder. The materials may be mixed together in any suitable manner, so that the binder will be interspersed with the particles of graphite. After the materials are mixed together, the mixture is placed in suitable molds adapted to produce the desired shape of finished brush or contact, and thereupon compressed by any means capable of exerting the necessary pressure, as, for example, by means of a 100 hydraulic press. In thus compressing the mixture, however, the pressure is exerted in a direction at right angles to a plane of the mass parallel to which it is desired to establish the path of least electrical resist- 105 ance. Very good results are obtained by

heating the molds, during the operation of compressing the mixture, to a degree sufficient to transform the binder into the desired final infusible and insoluble state. If 5 the mixture is compressed while cold, the heating and transformation of the binder into the desired infusible and insoluble state may be carried out in a suitable heater or oven.

10 The application of pressure, in the manner above described, that is, in a direction at right angles to a plane of the mass parallel to which it is desired to establish the path of least electrical resistance there- 15 through, tends to flatten out the flake-like conductive particles of graphite in planes or lines transverse or at right angles to the direction of the applied pressure, and even particles of granular conductive material 20 would have a tendency to thus flatten or crush down under the pressure exerted thereupon. As a consequence of this ten- 25 dency, the ends of adjoining particles would also tend, in many instances, to break the film of the binder at such ends and there- 30 upon make contact one with another, while the films of binder at the top and bottom sides would tend to remain intact. In any event, since by the flattening process, the 35 conductive particles have greater length and width than thickness, there would be, in the physical structure of the finished brush or contact, a larger number of insulating or high resistance films interposed between the 40 conductive particles in the direction of applied pressure, than would be interposed therebetween in a direction at right angles to the applied pressure. It follows there- 45 fore that the finished brush or contact body is given a novel internal physical structure which so modifies its electrical character- 50 istics as a conductor, that it possesses in predetermined lines or directions a high current carrying capacity of comparatively low resistance, while in lines or directions perpendicular thereto a comparatively high resistance is offered or interposed to the flow 55 of cross electric currents. A brush or contact device is thus provided which possesses 60 decidedly novel and advantageous electrical properties, especially when used for commutation purposes. The peculiar and novel internal physical structure, which character- 65 izes the brush or contact body, may not necessarily be in regular or symmetrical stratas, lines or layers, but it is, I believe, as above stated, a formation of comparatively free or uninterrupted conductive lines alternated more or less with lines of high 70 resistance or insulating effect, running, generally, in a given desired direction through the body of the brush or contact; and, fur- 75 thermore, it may be stated, as a rough de- 80 scription of such internal physical structure, that the conductive material and the non- 85

conductive or high resistance binder ma- 90 terial tends toward a stratified relative dis- position.

In the example above given, I have stated the proportions of conductive material relative to binder material to be nine to one, that is 90 per cent conductive material to 10 per cent of non-conductive or high resistance binder material. I do not wish to be understood, however, as thereby confining myself to the use of such specific relative proportions, since more or less variation either way as to the proportion of the binder material may be made, according to the tensile strength and carrying capacity it is 100 desired that the finished brush or contact shall possess. I have also found that 85 per cent of conductive material to 15 per cent of binder material forms a very satis- 105 factory brush for generator use, since it is of adequate physical strength and durability, while at the same time is electrically of comparatively high current carrying capacity. As a practical limiting range I prefer to use not more than 25 per cent of 110 the binder material, for beyond such proportion of non-conductive or high resistance binder, the electrical resistance becomes so high that the current carrying capacity is reduced beyond practical limits.

While it is preferable that the condensa- 115 tion product providing the binder element of the brush be solidified or hardened without carbonizing the same, whereby its inherent non-conductive or high resistance 120 electrical characteristics are unchanged, it may, nevertheless, be desirable in some instances and for certain specific uses to submit the brush to a heat sufficiently great to carbonize or partially carbonize the binder, 125 to thus produce a brush possessing a maximum current carrying capacity. In either case, however, the binder material formed from the described condensation products is 130 comparatively non-abrasive although adapted to reasonably resist wear, so that a brush containing the same is both strong and durable or long-lived.

I claim:—

1. An electrical brush or contact, comprising a mixture of a preponderance of electrically conductive material with a binder consisting of a relatively high resistance material capable of becoming insoluble and infusible when subjected to heat, said mixture being consolidated in such manner that the elements of the mixture are relatively dis- 135 posed to form an internal physical structure providing a path of least electrical resistance in lines substantially parallel to one plane of the mass.

2. An electrical brush or contact, comprising a mixture of electrically conductive material with between one and twenty-five per cent of a non-conductive or high resistance

binder consisting of a condensation product capable of becoming insoluble and infusible, said mixture being consolidated by pressure and heat.

- 5 3. An electrical brush or contact, comprising an electrically conductive material mixed with not to exceed approximately twenty-five per cent of a non-conductive or high resistance binder consisting of an infusible condensation product, said mixture being molded by pressure applied in one direction and solidified by heat, whereby the elements thereof are relatively disposed throughout the mass to form an internal physical structure having a path of least resistance substantially parallel to one plane of the mass.
- 10 4. An electrical brush or contact comprising graphite mixed with not to exceed approximately twenty-five per cent of an infusible and insoluble phenolic condensation product, said mixture being consolidated in such manner that the graphite and condensation product are relatively disposed throughout the mass to form
- 15 20 25 a substantially stratified internal physical

structure providing a path of least electrical resistance substantially parallel to one plane of the mass.

5. The process of manufacturing electrical brushes or contacts which consists in intimately mixing a dry comminuted conductive material with a relatively high resistance binder consisting of a condensation product capable of becoming insoluble and infusible, compressing the mixture by pressure applied in the direction of one axis of the mass, and solidifying the binder by heat.

6. The process of manufacturing electrical brushes or contacts which consists in mixing a dry comminuted conductive material with not to exceed approximately twenty-five per cent of a binder consisting of a condensation product capable of becoming insoluble and infusible, compressing the mixture by pressure applied in the direction of one axis of the mass, solidifying the binder by heat.

In testimony that I claim the invention set forth above I have hereunto set my hand this 28th day of August, 1922.

RALPH L. HENRY.